# EUROPEAN PATENT SPECIFICATION

(11) **EP 2 723 925 B1**
(45) Date of publication and mention of the grant of the patent: **11.10.2017**
(21) Application number: 12743876.0
(22) Date of filing: 22.06.2012
(51) Int. Cl.: D01D 7/00, D01D 5/00

(54) **A METHOD FOR PRODUCTION OF MATERIALS HAVING ANISOTROPIC PROPERTIES COMPOSED OF NANOFIBRES OR MICROFIBRES AND AN APPARATUS FOR IMPLEMENTATION OF SAID METHOD**
VERFAHREN ZUR HERSTELLUNG VON MATERIALIEN MIT ANISOTROPEN EIGENSCHAFTEN AUS NANOFASERN ODER MIKROFASERN UND VORRICHTUNG ZUM DURCHFÜHREN DES VERFAHRENS
PROCÉDÉ DE PRODUCTION DE MATÉRIAUX PRÉSENTANT DES PROPRIÉTÉS ANISOTROPES ET COMPOSÉS DE NANOFIBRES OU DE MICROFIBRES, ET APPAREIL POUR METTRE EN OEUVRE LEDIT PROCÉDÉ

(30) Priority: 27.06.2011 CZ 20110376
(43) Date of publication of application: 30.04.2014
(73) Proprietor: Contipro Biotech s.r.o., 56102 Dolni Dobrouc (CZ)
(72) Inventor: POKORNY, Marek, 561 64 Jablonne nad Orlici (CZ); MARTINCOVA, Lada, 517 41 Kostelec nad Orlici (CZ); VELENBY, Vladimir, 564 02 Zamberk (CZ)
(74) Representative: Zemanová, Veronika
(86) International application number: PCT/CZ2012/000055
(87) International publication number: WO 2013/000442

(56) References cited:
- EP-A1- 2 045 375
- WO-A1-2011/095141
- GB-A- 480 950
- US-A1- 2010 327 494
- KATTA P ET AL: "Continuous Electrospinning of Aligned Polymer Nanofibers onto a Wire Drum Collector", NANO LETTERS, ACS, US, vol. 4, no. 11, 28 September 2004 (2004-09-28), pages 2215-2218, XP002466227, ISSN: 1530-6984, DOI: 10.1021/NL0486158 cited in the application
- M. POKORNY ET AL: "Collection method for extra aligned nanofibers deposited by electrospinning", REVIEW OF SCIENTIFIC INSTRUMENTS, vol. 82, no. 5, 1 January 2011 (2011-01-01), page 055112, XP55041388, ISSN: 0034-6748, DOI: 10.1063/1.3592596
- AKBAR JAFARI ET AL: "Well-aligned Nano-fiberous Membranes Based on Three-pole Electrospinning with Channel Electrode", MACROMOLECULAR RAPID COMMUNICATIONS, vol. 32, no. 12, 5 May 2011 (2011-05-05), pages 921-926, XP55041383, ISSN: 1022-1336, DOI: 10.1002/marc.201100101
- YUUKI KARUBE AND HIROYOSHI KAWAKAMI: "Fabrication of well-aligned electrospun nanofibrous membrane based on fluorinated polyimide", POLYMERS FOR ADVANCED TECHNOLOGIES, WILEY & SONS, BOGNOR REGIS, GB, 1 January 2009 (2009-01-01), pages 1-6, XP007914971, ISSN: 1042-7147, DOI: 10.1002/PAT.1511 [retrieved on 2009-07-16]

## Description

### TECHNICAL FIELD OF THE INVENTION

The present invention relates to a method for production of two-dimensional or three-dimensional fibrous materials of microfibres or nanofibres in which at first nanofiber or microfiber is continuously drawn out of a solution, which nanofibre or microfibre is pulled to a rotary set of *n* electrodes by means of electrostatic field. In the process individual electrodes are arranged at regular spacing to each other and at the same distance from the set of electrodes rotation axis and parallel with it. This set of electrodes rotates and thereby the nanofibre or microfibre is wound on it. After the nanofibre or microfibre was wound the electrostatic field is disconnected and rotation of the electrode set is stopped, and a layer of microfibres or nanofibres formed in the field between two adjacent electrodes is removed. The invention also refers to an apparatus for production of the two-dimensional or three-dimensional fibrous materials of microfibres or nanofibres. This apparatus includes at least one spinning nozzle attached to a first potential and a set of electrodes facing the nozzle arranged at regular spacing to each other and attached to a second potential. Further it includes an accumulator for collecting microfibres and nanofibres settled between couples of adjacent electrodes.

### BACKGROUND OF THE INVENTION

Production of microfibres or nanofibres is implemented by a method of electrostatic spinning. This method is presented as "Electrospinning" in professional literature. In this method the forming of melt or solution of polymers into fibrous structures is brought about by effects of high electrostatic field. Forces of this field at first give rise to a spurt of a trickle out of the polymer solution or melt droplet and then they activate also its movement to an opposite electrode. During the movement a thinning, drawing and solidification of the polymer occur and the polymer in the solid fibres form falls on the opposite electrode, so-called collector. The whole of this fibre movement between the two electrodes is highly complicated and its trajectory is quite random. Literally chaotic movement of the flying fibre gives rise to its random depositing on the opposite electrode, where a nonwoven fibrous material with fibres having their diameter from ten nanometres to tens of micrometres is formed. This manufacturing method is known from US patent US2048651.

Nano-fibrous or micro-fibrous materials with highly fine structure find numerous applications in many fields of advanced medicine, but also of microelectronics, optics and power engineering. Huge surface formed in relatively very small volume is one of the basic advantages of these materials, and inter-fibre spaces (pores) of these materials have very small size. Material with fine internal nano-structure or microstructure assumes quite new properties that can be considerably different from properties of a volume sample of the same material. Additionally it is possible to control these unique properties and adapt them to requirements of particular application by a controlled production. Future applications count on a use of such materials in various fields of advanced medicine, because such material provides cells in living tissue with very favourable and natural conditions for their growth, motion and reproduction. Unfortunately the usability of such material is considerably limited just because of its internal chaotic structure. Applications of tissue engineering specify their requirements on regular 3D structures that are subsequently used as replacements of cartilages, bones, and nerve, vascular and cardiovascular transplants and the like. Just an internal axial orderliness of material considerably supports directional growth and motion of cells, tissues, and also supports regeneration of long nervous disorder. The ordered structure ensures required flexibility of the material when stressed in applications such as muscular and connective tissues replacements. Mechanical properties of the material can be quite well controlled just by choice of the internal structure axial orderliness. Need of new materials with precise internal morphology is required by numerous applications not only in the field of advanced medicine. The regular structure is quite essential also e.g. for miniature electronic or optical connections that can be provided by nanofibres or microfibres produced by the method disclosed in this invention.

Current methods and production techniques of the oriented nanofibres or microfibres are solved by means of rotating collector that is driven at high revolutions. Surface of such collector, in most cases in the shape of a cylinder or a thin rod as described in US4552707 or US20020084178, captures flying fibre and mechanically carries it in the direction of the collector own movement; the fibre is practically wrapped around the rotating cylinder. Nanofibres or microfibres are deposited directly onto the cylinder surface or are formed in a gap between two rotary rods that are positioned on one rotation axis, see US20070269481. Surface of such collector is one of the electrodes and thus it must be made of a conductive material. Unless the collector is directly connected to one of high-voltage power supply poles, see US20090108503, US4689186, or if its surface is overlapped with non-conductive substrate, significant losses of the production process efficiency arise, because practically an insulating material is inserted between two main electrodes and thus electric field is degraded and its homogeneity is disturbed. Reduced efficiency is indicated with longer deposition of fibres, because the thicker deposited layer acts also as an undesirable insulant and thus further fibres are repelled in a different direction from the collector. In the area of so far deposited fibres a charge is accumulated that has the same polarity as a charge carried by a fibre before its impact on the collector. Repulsive forces act between these charges of the same polarity, which forces influence negatively the ordering of newly deposited fibres. The negative effects of this charge are increased, when thicker fibrous layers are deposited, because fibres in upper layers are already deposited randomly and no longer respect the axial orderliness as it is with fibres deposited in lower layers. Furthermore the resulted fibrous layer has a partially limited degree of order, which is caused by capturing the flying fibre having direction different from just perpendicular to the surface of the rotating cylinder. On principal the methods mentioned above function well, however results, with regard to achieving precise orientation of the internal structure of the fibrous materials, are generally unsatisfying, because there is still high percentage of fibres in produced materials that do not respect any of preferred directions.

Subsequent manipulation with the fibrous material and its controlled taking off from the collector surface is quite essential problem that is not a part of any of contemporary technical solutions. The fibrous layer is deposited onto the collector and for its subsequent use it must be transferred usually onto quite different underlayment or into another container, etc. And so manually one by one cut out stripes of fibrous material are assembled in thicker 3D structures in examples of embodiments disclosed in patent application US20080208358A1. Such a layer is highly fine and a manipulation with the nano-fibrous or micro-fibrous material is complicated, because an irreversible damage of the layer arises very easily already when being taken off from the collector used. Any manipulation with material of a larger area is almost impossible especially with bio polymeric fibres with very low mechanical resistance. Currently there is no mechanisms solved, which would provide suitable mechanical manipulation and transfer of nano-fibrous or micro-fibrous layer onto another, i.e. any underlayment while maintaining or even increasing of the orientation degree of the fibres in the layer.

Patent application WO2006136817A1 describes a use of a rotating collector with electrodes longitudinally arranged around an axis of rotation. Geometric dimensions of the collector are not mentioned. Authors give no method for taking off fibres from the collector carefully. No collecting mechanism for fibres deposited onto the rotating collector is solved. The described method does not solve all phases of the production process or more precisely the process is terminated by the fibres deposition. Therefore it is impossible to finish the production process without an operator intervention and manual manipulation, which results in considerable decreasing of quality and internal structure of the material.

In publication of Katta et al. (Katta P., M. Alessandro et al. NanoLetters, 4(11): 2215-2218, 2004) rotating cylinder built-up of longitudinal conductive electrodes as a collector for creating oriented fibres is used. The collector with approximately forty conductive electrodes, which are distant 10 mm from each other and create the rotating collector with diameter of 120 mm, is described in the publication. A loss of uniaxial fibres orientation during longer time deposition is demonstrated here. Optimization and description of parameters important for operational utilization are not carried out here. The authors also do not mention further steps for processing of the fibrous layer deposited onto this type of collector. Published patent application EP2045375 A1 discloses a method and apparatus for the production of two- and three-dimensional fibrous materials, wherein aligned electrospun fibres are deposited between two rotating parallel circular electrodes. The fibrous material is formed by consecutive removal of fibres from between the conductive electrodes onto an accumulator.

A publication of Pokorny et al. (P. Pokorny and V. Velebny, Review of Scientific Instruments, 82, number 055112, 2011) discloses a method and apparatus wherein consecutive layers of aligned electrospun fibres are collected by multiple sweeping of an accumulator over the same electrode pair.

### SUMMARY OF THE INVENTION

Drawbacks of state of the art mentioned above are eliminated to a considerable extent by a method of production of two-dimensional or three-dimensional fibrous materials of fibres with a diameter of microfibres or nanofibres according to the invention, in which at first nanofibre or microfibre is continuously drawn out of a solution, which nanofibre or microfibre is pulled to a rotary set of *n* electrodes (where *n* is a natural number from 1 to 200) by means of an electrostatic field. Individual electrodes of the set are arranged at regular spacing to each other and at the same distance from the set of electrodes rotation axis and parallel with it. This set of electrodes rotates and thereby the nanofibre or microfibre is wound on it. After the nanofibre or microfibre thin layer was formed the electrostatic field is disconnected and rotation of the electrode set is stopped, and a layer of microfibres or nanofibres formed in the field between two adjacent electrodes is removed. Afterwards the rotary set of electrodes turns through an angle of *360*/*n* and the layer of microfibres or nanofibres formed between two adjacent electrodes in the field adjacent to the field, from which a layer was removed in previous step, is removed. This step is repeated n-times till layers of microfibres or nanofibres from all the fields between adjacent electrodes are removed.

In an advantageous embodiment of the method according to the invention, before the layer of microfibres or nanofibres is removed from a new field, an accumulator turns around slightly to reach a direction of microfibres or nanofibres in the removed layer that is different from the direction of microfibres or nanofibres of the preceding layer.

In another advantageous embodiment of the method according to the invention superimposed layers of microfibres or nanofibres are pressed together, whereas by pressing the layers together it is possible simultaneously to form a required three-dimensional shape of the final product. An article formed in this way can be embedded with another medium to create a composite material of required properties.

Drawbacks of the state of the art mentioned above are eliminated to a considerable extent even by an apparatus for production of two-dimensional or three-dimensional fibrous materials of microfibres or nanofibres comprising at least one spinning nozzle connected to a first potential and a set of *n* electrodes facing the spinning nozzle that are arranged at regular spacing and connected to a second potential, and also an accumulator for collecting microfibres or nanofibres settled between two adjacent electrodes. The set of the electrodes is pivoted in this apparatus and individual electrodes of the set of the electrodes are arranged at regular spacing to each other and at the same distance from the set of electrodes rotation axis and parallel with it. The apparatus further comprises the accumulator, which is arranged, in relation to the electrodes, movably in direction of longitudinal axes of the electrodes, for collecting microfibres or nanofibres settled between two adjacent electrodes. Furthermore this accumulator is arranged, in relation to the electrodes, movably in direction perpendicular to the longitudinal axes of the electrodes for it being brought into engagement to collect microfibres or nanofibres settled between two adjacent electrodes, and being brought out of engagement after finishing the collection of microfibres or nano fibres settled between two adjacent electrodes.

In an advantageous embodiment of the apparatus according to the invention the accumulator has a shape of parallelogram, the width of which is smaller than a distance between nearest surfaces of a couple of adjacent electrodes to enable its insertion between said adjacent electrodes.

In another advantageous embodiment of the apparatus according to the invention the accumulator is arranged rotationally around a line perpendicular to the surface of the collector and passing through the centre of the collector surface in order that the accumulator may turn around slightly to place a further layer of microfibres or nanofibres settled between two adjacent electrodes with direction of microfibres or nanofibres that is different from the direction of microfibres or nanofibres of the preceding layer.

In another advantageous embodiment of the apparatus according to the invention the accumulator has a shape of square with its side shorter than a distance between nearest surfaces of a couple of adjacent electrodes, the accumulator being arranged rotationally around a line perpendicular to the surface of the collector and passing through the centre of the collector surface in order that the accumulator may turn through an angle of 90° to place a further layer of microfibres or nanofibres settled between two adjacent electrodes with direction of microfibres or nanofibres that is perpendicular to the direction of microfibres or nanofibres of the preceding layer.

In yet another advantageous embodiment of the apparatus according to the invention the accumulator is made in the form of a dish for depositing the collected layers of nanofibres or microfibres, the apparatus being further provided with a piston for compression of the fibres into the accumulator and for compaction of individual collected layers of nanofibres or microfibres to mechanically strengthen ordered 3D structure. In such a case it is also advantageous if the accumulator is arranged rotationally around a line perpendicular to the surface of the collector and passing through the centre of the collector surface in order that the accumulator may turn around slightly to place a further layer of microfibres or nanofibres settled between two adjacent electrodes with direction of microfibres or nanofibres that is different from the direction of microfibres or nanofibres of the preceding layer.

### BRIEF DESCRIPTION OF THE DRAWINGS

The subject matter of the invention is described in details with reference to the accompanying drawings. Fig. 1 is a flow chart of particular phases of the production process as suggested in solution according to the present invention. Fig. 2 represents an exemplary embodiment of an apparatus for the production of fibrous materials with anisotropic properties, while the shown accumulator is not of a type covered by the claims. Side sectional elevation of longitudinal electrodes of a rotating collector with accumulator is on Fig. 3, and further exemplary embodiment is on Fig. 4a. Fig. 4b shows a cross section of four and five longitudinal electrodes of a rotating collector, whereas principal of parallel ordered fibres formation is depicted. In a similar way principal of the production of perpendicular fibres in two steps with exemplary use of four and five longitudinal electrodes of the rotating collector is shown on Figs. 5a and 5b. Photos of parallel and perpendicular ordered fibres from an electron microscope are on Figs. 6 and 7.

### DETAILED DESCRIPTION OF THE INVENTION

It is the aim of the present invention to accomplish the production of nano-fibrous or micro-fibrous materials with high degree of areal (2D) and volume (3D) internal ordering that can be controlled by changing process parameters for the purpose of controlling morphological and anisotropic properties of the resulting materials. Furthermore it is also the aim of the present invention to solve suitable mechanical manipulation and transfer of the new material onto any underlying or also packing material, whereas the order degree of internal structure of the material is maintained. In an advantageous embodiment of the invention a movable accumulator 7 is a suitable dish that enables easy further treatment of the fibrous material (e.g. in production of composite materials).

The subject matter of the invention is a comprehensive production process of new materials that is divided into particular process phases, the exemplary sequence of which is shown on Fig. 1. A spinning mixture is prepared in the first step. Subsequently the solution or melt 1 is measured out into a spinning nozzle 3, after which a high electric voltage is connected, which gives rise to a fibre 5 with a diameter ranged from microfibres to nanofibres. The fibre 5 moves in the electrostatic field in the direction to a collector 9. Fibres 5 are deposited onto the rotating collector 9 in one preferred direction. After a layer 8 of fibres 5 was created on the collector, the deposited fibres 5 are collected and layers 8 of these fibres 5 are in turn superimposed, while the degree of their order is maintained. Thereafter the fibre layers 8 are compressed, through which a finished product that can be enfolded in a wrapping material, or a semi product intended for further processing such as an application of suitable medium so that the resulted product may be a composite material and gain required properties, comes into existence. It is possible to enfold the finished product in the wrapping material with the shape of a tray that makes manipulation easier and is also suitable for subsequent treatments of fibre layers 8 such as embedding the layer 8 of fibres 5 with another medium in order to get a composite material, and thus a final product comes into existence. Removing and transfer of the product is a final phase. Advantageously all of these phases are implemented automatically in a deposition chamber without any intervention of an operator and without being affected by external environment, which makes it possible to ensure the process sterility and a high quality of final products. The production process phases are represented in the flow chart on Fig. 1, where repeated process phases are also indicated. The process is repeated from the beginning unless a sufficient layer 8 of fibres 5 is collected by the accumulator 7 at the moment of solution 1 reserve exhaustion in phases "Fibres deposition" or "Superimposing".

An exemplary embodiment of an apparatus for production of two-dimensional or three-dimensional fibrous materials composed of nanofibres or microfibres, hereinafter referred to as fibres 5, is on Fig. 2. This apparatus comprises a jet emitter 2 filled with solution 1 of polymer and equipped with spinning nozzle 3. In spite of the fact that for simplicity's sake only one jet emitter 2 is depicted on Fig. 2, it is obvious that there will be more such jet emitters 2 in actual apparatus. The spinning nozzle 3 is connected to a first potential, i.e. to one of poles of a source 4 of DC electric voltage. The second pole of the source 4 of DC electric voltage is connected to the collector 9 facing the spinning nozzle 3. The collector 9 is composed of electrodes 6 that are arranged longitudinally at regular spacing to each other and at the same distance from the collector 9 rotation axis x. The accumulator 7 is arranged movably, in relation to the electrodes 6, in direction parallel with the rotation axis x of the collector 9 so that the accumulator 7 may collect layers 8 of fibres 5 settled between two adjacent electrodes 6. The accumulator 7 shown in Fig. 2 is not of a type covered by the claims.

Fig. 3 schematically depicts a side view of an accumulating mechanism with the planar accumulator 7. Fibres 5 are deposited by electrostatic spinning onto the electrodes 6 of the collector 9. Afterwards the fibres 5 are deposited onto a surface of the accumulator 7 while their order is maintained. In this exemplary embodiment the accumulator 7 is planar. It is inclined in relation to the rods of the electrodes 6 of the collector 9 at an angle *α*, and moves in translatory movement in the direction that forms an angle β with the axis *x* of the collector.

Fig. 4a schematically depicts a cross-section of the collector 9 with four electrodes 6 and the accumulator 7. Fibres 5 are deposited by electrostatic spinning on the conductive rods of the electrodes 6 of the collector 9. Afterwards the fibres 5 are deposited on a surface of the accumulator 7 while their order is maintained. The collector 9 is equipped with four electrodes 6. The squared accumulator 7 removed a layer 8 of fibres 5 from the field between two upper electrodes. On the right the subsequent phase is depicted, where the collector 9 is turned through an angle of 90° and the accumulator 7 removes another layer 8 of fibres 5 with the same orientation.

Fig. 4b schematically depicts a cross-section of the collector 9 with five electrodes 6 and the accumulator 7. Fibres 5 are deposited by electrostatic spinning onto the conductive rods of the electrodes 6 of the collector 9. Afterwards the fibres 5 are deposited on a surface of the accumulator 7 while their order is maintained. The collector 9 is equipped here with five electrodes 6. The squared accumulator 7 removed a layer 8 of fibres 5 from the field between the two upper electrodes. On the right the subsequent phase is depicted, where the collector 9 is turned through an angle of 360/5, i.e. 72° and the accumulator 7 removes another layer 8 of fibres 5 with the same orientation. There are two layers 8 of fibres 5 with the same orientation on the accumulator 7.

Fig. 5a schematically depicts a cross-section of the collector 9 with four electrodes 6 and the accumulator 7. Fibres 5 are deposited by electrostatic spinning on the conductive rods of the electrodes 6 of the collector 9. Afterwards the fibres 5 are deposited on the surface of the accumulator 7, while their order is maintained. The collector 9 is equipped with four electrodes 6. The squared accumulator 7 removed a layer 8 of fibres 5 from the field between the two upper electrodes. On the right the subsequent phase is depicted, where both the collector 9 and the accumulator 7 are turned through an angle of 90° and the accumulator 7 removed another layer 8 of fibres 5. Thus there are two layers 8 of fibres 5 on the accumulator 7, whereas the orientation of fibres 5 of the first layer 8 is perpendicular to the orientation of fibres 5 of the second layer 8.

Fig. 5b schematically depicts a cross-section of the collector 9 with five electrodes 6 and the accumulator 7. Fibres 5 are deposited by electrostatic spinning onto the conductive rods of the electrodes 6 of the collector 9. Afterwards the fibres 5 are deposited on the surface of the accumulator 7, while their order is maintained. The collector 9 is equipped here with five electrodes 6. The squared accumulator 7 removed a layer 8 of fibres 5 from the field between the two upper electrodes. On the right the subsequent phase is depicted, where the collector 9 is turned through an angle of 360/5, i.e. 72°, and the accumulator 7 is turned through an angle of 90° and removes another layer 8 of fibres 5. Thus there are two layers 8 of fibres 5 on the accumulator 7, whereas the orientation of fibres 5 of the first layer 8 is perpendicular to the orientation of fibres 5 of the second layer 8.

Fig. 6 is a photo from an electron microscope at magnification 5000-times, where several layers 8 of fibres 5 superimposed with the same orientation are depicted.

Fig. 7 is a photo from an electron microscope at magnification 1000-times, where several layers 8 of fibres 5 are depicted, whereas layers 8 were superimposed in such a way that the orientation of fibres 5 of one layer 8 is perpendicular to the orientation of fibres 5 of the previous layer 8.

In operation of the apparatus for production of the two-dimensional or three-dimensional fibrous materials a prepared spinning mixture is dosed into the jet emitter 2. Afterwards a high electric voltage is connected and it causes that the solution or melt begins to escape out of the spinning nozzle 3 creating fibre 5 with diameter ranging from microfibres to nanofibres. This fibre 5 moves in the electrostatic field in the direction to the collector 9. The fibres 5 are deposited onto the rotating collector 9 in one preferred direction. After the layer 8 of the fibres 5 was formed on the collector 9, high electric voltage is disconnected and the fibre 5 quits escaping out of the spinning nozzle 3. Thereafter the accumulator 7 collects the settled fibres 5, and the layers 8 of these fibres 5 are step by step superimposed, while their degree of order is maintained. According to requirements on the resulted material, the layers 8 of the fibres 5 are superimposed so that the fibres 5 orientation may be the same in all layers, or it is possible to turn the orientation of the fibres 5 in each subsequent layer 8 through an angle, usually through 90°. After a sufficient number of the layers 8 was superimposed it is possible to compress the fibrous layers 8 and thus either a final product, that can be enfolded in a wrapping material, or a semi product intended for further processing such as an application of suitable medium so that the resulted product may be a composite material and gain required properties, comes into existence.

It is an advantage of this embodiment that the fibres 5 deposited onto the surface of the accumulator 7 have a higher degree of order than fibres 5 settled onto a surface of a rotating cylinder because further straightening of them in one direction occurs just by a movement of the accumulator 7. Thus the degree of order of the internal fibrous material structure is higher than that of the material that was formed on the surface of the rotating cylinder.

Another advantage of this embodiment, when compared with stationary segmented collector with planar electrodes, is multiple lengths of ordered nanofibres, which enables to produce materials of larger area or volume with very well ordered internal structure. At very low revs of the collector 9 first of all electrostatic forces, which act transversely between particular electrodes 6 of the collector 9, contribute to the fibre 5 orientation. On the contrary at high revs even mechanical forces, which capture flying fibre 5 and attract it to the electrodes 6 of the collector 9 namely in one direction, i.e. perpendicular to the electrodes 6, join the electrostatic forces contributing to ordered depositing of the fibres 5 onto the collector 9. That way both the important components of forces - electrostatic and mechanical - are added up and thus the resulted degree of uniaxial order of the fibres 5 is multiplied. This principal is proved by long-term experimental and theoretically supported results that demonstrate formation of very well oriented fibres 5 of a diameter ranging from microfibres to nanofibres with multiply longer length when using segmented rotating collector 9, than when using stationary segmented collector of similar geometrical parameters. In order that a very good orientation of fibres 5 may be reached, revolutions of the collector 9 described in this patent application are set to a value by several tens of percent lower, than a minimal revolutions of a cylinder with the whole of conductive surface, namely just because of the contribution of electrostatic forces. Reduction of rotating speed leads to steadier air flow, which arises around fast rotating collector 9 and which pulls flying fibres 5 in uncontrolled direction.

Yet another advantage is the possibility of implementation of all the production cycle phases in a single closed apparatus, namely in a deposition chamber, where an automatic production without an operator intervention and without being influenced by external environment is ensured, which enables to ensure the process sterility and a high quality of resulting products.

In an advantageous embodiment of this apparatus the rotating collector 9 with the set 11 of the electrodes 6 connected to the second potential comprises at least three longitudinal electrodes 6, generally N electrodes 6, and the accumulator 7 that moves successively always between two adjacent electrodes 6 in such a way, that the accumulator 7 movement direction is determined by combining a movement in direction of the common axis *x* of rotation of the electrodes 6 of the collector 9, and a movement in direction that forms with the axis *x* a specified angle β. The accumulator degree of incline is defined by an angle *α*. In a plane transverse to the set 11 of the electrodes 6 an angle *γ* is defined, which specifies an angular displacement of the accumulator and the collector 9 to each other. The next collection of the fibres 5 is performed after turning the electrodes 6 of the collector in relation to the accumulator through an angle *γ* = 360/N.

In another exemplary embodiment of this apparatus the rotating collector 9 with electrodes 6 connected to the second potential includes at least three longitudinal electrodes 6, generally *N* electrodes 6, and the accumulator 7 that moves successively always between two adjacent electrodes 6 in such a way, that the next collection of fibres is performed after turning the electrodes 6 of the collector 9 in relation to the accumulator 7 through an angle *γ* = 90 + 360/N. However in this case between two consecutive collections of the layers 8 of the fibres 5 the accumulator 7 turns around its axis perpendicular to the surface of the accumulator 7, which is squared in this case, through an angle of 90°. That way the fibres are deposited in individual layers, where fibres in one layer are perpendicular to fibres of preceding layer.

Yet another exemplary embodiment of the apparatus comprises the rotating collector 9 with four longitudinal electrodes 6, and the accumulator 7, which moves in a direction perpendicular to said electrodes 6 axes for enabling of an insertion of inclinable plates of the accumulator 7 between said neighbouring electrodes 6 and their release and in the lengthwise direction along the electrodes 6. The accumulator 7 is provided with four said inclinable plates capturing on their surfaces fibres 5 settled between two closest adjacent electrodes 6. After capturing of fibre layers on said inclinable plates of the accumulator 7 said inclinable plates, one after the other, are tilted 180° along the edge of the inclinable plate that is closest to the longitudinal axis of the collector 9 and the fibre layer from the inclinable plate is captured on the collecting plate that is perpendicular to the longitudinal axis of the collector 9. Thus after subsequent capturing of individual fibre layers from the subsequent inclinable plates four fibre layers laid on each other are created, the fibres 5 of each layer being perpendicular to the neighbouring layer.

Very effective drying or solidification of the fibres 5 and effective evaporation of a solvent, that is moreover not collected in vicinity of the collector 9, are also advantages of the rotating collector 9 with longitudinal electrodes 6. This has an essential influence on a diameter of the fibres 5 that are formed between electrodes 6 of the collector 9. Their diameter can be reduced by setting the parameters of the process.

In another advantageous embodiment of this apparatus the collector 9 is comprised of more than three conductive electrodes 6 that are arranged at regular spacing to each other and at the same distance from a common rotation axis x. The accumulator 7 has a shape of a disc and is provided with appropriate notches that enable sliding the accumulator onto the longitudinal electrodes 6 so that its movement along the rotation axis x and in the vicinity of these electrodes 6 may be enabled. During this movement, fibres 5, which were deposited in an orderly manner between adjacent electrodes 6, are placed spontaneously directly onto a surface of the accumulator 7, where stripes of new material are formed, which stripes are composed of uniaxial ordered fibres 5 with high degree of orientation.

Another advantageous embodiment comprises the cylindrical collector 9 composed of at least two longitudinal electrodes 6, generally of total number of *N*, where N is a natural number, parallelly arranged electrodes, the distance of which ranges from 0.1 mm to *(π.d*/*N)* mm, where *d* is double distance of the electrodes 6 from the common rotation axis *x*. In the first limit case very thin conductive wires are used as the electrodes 6, in the second limit case - not covered by the claims - the electrodes 6 form an integral conductive surface of the cylinder. In the first limit case fibres 5 are captured onto the very thin electrodes 6 and resulting material is composed of very well ordered fibres 5 only, the fibres having their diameter ranging from microfibres to nanofibres. In the second limit case fibres 5 are wiped off in the same way as above mentioned, whereas during the fibres 5 depositing a yarn or a filament is formed that is composed of multiple fibres 5 with a total length of *π.d.*

Finally in yet another advantageous embodiment of this apparatus the accumulator 7 has a shape of a dish for accumulating the collected layers 8 of fibres 5. The fibres 5 are compressed into the accumulating dish by means of a simple piston motion. Individual layers 8 are compacted in the dish and that way the ordered 3D structure is also mechanically strengthened. The dish serves for further treatment of the product, e.g. by imbedding fibres 5 with another solution, generally with another medium, a composite material of required properties is produced.

Hereinafter concrete exemplary embodiments of the apparatus according to the present invention will by described.

### Example 1: Fibrous layer composed of parallel fibres.

Fibres of 16% aqueous solution 1 of polyvinyl alcohol (PVA) were extruded from a jet emitter 2 through a spinning nozzle 3, and deposited onto a segmented collector 9 (Fig. 2). The electrodes 6 of the collector 9 were distant 12 cm vertically from the spinning nozzle 3. The collector 9 was provided with four longitudinal electrodes 6 in the shape of thin wires of a circular cross-section with a diameter of 0.8 mm. The electrodes 6 distances were 25 mm to each other. By means of a low DC voltage source the collector 9 was set spinning at 2000 revs per minute, which corresponds to the collector linear surface speed of 3.7 meter per minute. Another source 4 of high voltage was connected between the spinning nozzle 3 and the collector 9 and its output was set to 28 kV. Electrostatic forces gave rise to a formation of a fibre 5 with a diameter ranging from microfibres to nanofibres, which fibre was in turn deposited between the electrodes 6 in the form of a layer 8 of the ordered fibres 5. After 30 seconds the fibre 5 depositing was interrupted and the rotating collector was stopped or a power supply of the collector 9 motor and the high voltage source 4 were switched off. Afterwards the layer 8 of the fibres 5 was wiped off by a slow motion *v(t)* of the accumulator 7 along the electrodes 6 of the collector 9, whereas the accumulator 7 was inclined at an angle of α = 75°. Side view of this arrangement is depicted in Fig. 3. After the first layer 8 of fibres 5 had been deposited onto the accumulator, the collector 9 was turned through an angle of 90°. At a successive movement of the accumulator 7 another layer 8 of the fibres 5 was deposited onto its surface. This process was repeated until all the fibres 5, deposited among the four longitudinal electrodes 6, were collected (Fig. 4a). After that the spinning was started again and the whole process was repeated. By repeating this process it is possible to produce a layer of almost any thickness on the area of (25x25) mm². A surface of such a layer is shown in Fig. 6, which is a photo from electron microscope at magnification 5000-times. The spinning took place under laboratory conditions - temperature 24°C and relative humidity 40%.

### Example 2: Material with regular 3D structure composed of fibres perpendicular to each other

Fibres 5 of a diameter ranging from microfibres to nanofibres were deposited onto the rotating collector 9 with four longitudinal electrodes in the same way as mentioned in example 1. After stopping the spinning process and the rotating collector 9, the fibres 5 were wiped off by the accumulator 7 (Fig. 5a). The accumulator 7 was in motion along the conductive rodlike electrodes 6 of the collector 9 so that the first layer of the fibres 5 was formed on a surface of the accumulator 7. Afterwards the whole collector 9 turned through an angle of 90° and simultaneously also the squared accumulator 7 sized 25x25 mm turned through an angle of 90°. The accumulator 7 was set in motion along the conductive rodlike electrodes 6 of the collector 9, during which time the second layer of fibres 5 was being deposited. The fibres 5 in the second layer 8 were deposited perpendicularly to the fibres 5 of the first or the preceding layer 8. This process was repeated four times until all the fibres 5 were wiped off the collector 9. Thereafter the collector 9 was set spinning and the spinning process was started. The sample produced by this process has a regular 3D structure of an area of (25x25) mm². An example of such material surface is shown in Fig. 7, which is a photo from electron microscope at magnification 1000-times.

### INDUSTRIAL APPLICABILITY

The present invention can be used for production of materials that are areal (2D) or voluminous (3D) from the macroscopic point of view, and which are composed of nanofibres or microfibres, whereas the internal fibrous structure of these materials is regular, ordered in one direction or in more directions.

## Claims

1. A method of production of two-dimensional or three-dimensional fibrous materials of fibres (5) arranged in preferred directions, the fibres (5) being of a diameter ranging from microfibres to nanofibres, where in step a)
- the fibre (5) is continuously drawn out of a solution (1) or melt, and pulled to a rotary set (11) of *n* conductive electrodes (6), where *n* is a natural number, by means of an electrostatic field, the individual electrodes (6) of the set (11) being arranged at regular spacing to each other and at the same distance from the set (11) of electrodes (6) rotation axis and parallel with it, the fibre (5) being wound on the set (11) of the electrodes (6) by rotating the set (11) of the electrodes (6), after which in step b)
- the electrostatic field is disconnected and rotation of the set (11) of the electrodes (6) is stopped, and a layer (8) of the fibres (5) formed in the field between two adjacent electrodes (6) is removed,
**characterised in that** in the subsequent step c)
- the rotating set (11) of the electrodes (6) turns through an angle of 360/n, the layer (8) of the fibres (5), formed between two adjacent electrodes (6) in the field adjacent to the field from which the layer (8) was removed in preceding step b), is removed, and this step is repeated in total n-times.

2. The method of claim 1 **characterised in that** before the step c), where the layer (8) formed in the field between two adjacent electrodes (6) is removed, the accumulator (7) turns round slightly to reach the fibres (5) direction different from the fibres (5) direction of the preceding layer (8).

3. The method of claim 1 **characterised in that** the superimposed layers (8) of the fibres (5) are pressed together.

4. The method of claim 3 **characterised in that** a required spatial shape of final product is formed by compressing the layers (8) of the fibres (5).

5. The method of claim 4 **characterised in that** the object formed of the fibres (5) is imbedded with another medium, thus creating a composite material of required properties.

6. An apparatus for the production of two-dimensional or three-dimensional fibrous materials of the fibres (5) for implementation of the method of claims 1 to 5, comprising at least one spinning nozzle (3) connected to a first potential and a set (11) of conductive electrodes (6), facing the nozzle, arranged at regular spacing to each other and attached to a second potential, and an accumulator (7) for collecting fibres (5) settled between two adjacent electrodes (6), individual electrodes (6) of the set (11) of the electrodes (6) are arranged at regular spacing to each other and at the same distance from the set (11) of electrodes (6) rotation axis and parallel with it, **characterised in that**
- the apparatus is adapted to rotate the set (11) of the electrodes (6) during step a) and to turn the set (11) through an angle of 360/n during step c), n being the number of electrodes (6) within the set (11) and
- whereas the accumulator (7)
- is, in relation to the electrodes (6), arranged movably in the direction of longitudinal axes of the electrodes (6) for collecting the fibres (5) settled between two adjacent electrodes (6), and
- is, in relation to the electrodes (6), arranged movably in the direction perpendicular to the longitudinal axes of the electrodes (6) for it being brought into engagement to collect fibres (5) settled between two adjacent electrodes (6), and being brought out of engagement after finishing the collection of fibres (5) settled between two adjacent electrodes (6).

7. The apparatus of claim 6 **characterised in that** the accumulator (7) has a shape of parallelogram, the width of which is smaller than a distance between nearest surfaces of a couple of adjacent electrodes (6) to enable its insertion between said adjacent electrodes (6).

8. The apparatus of claim 7 **characterised in that** the accumulator (7) is arranged rotationally around a line perpendicular to the surface of the accumulator (7) and passing through the centre of the accumulator (7) surface for depositing the subsequent layer (8) of the fibres (5) settled between two adjacent electrodes (6) with the fibre (5) direction different from the direction of the fibres (5) of the preceding layer (8).

9. The apparatus of claim 7 **characterised in that** the accumulator (7)
- has a squared shape with its side shorter than a distance between nearest surfaces of two adjacent electrodes (6), and
- is arranged rotationally around a line perpendicular to the surface of the accumulator (7) and passing through the centre of the accumulator (7) surface for turning the accumulator (7) through an angle of 90° for depositing the subsequent layer (8) of the fibres (5) settled between two adjacent electrodes (6) with the fibres (5) direction perpendicular to the direction of the fibres (5) of the preceding layer (8).

10. The apparatus of claim 6 **characterised in that** the accumulator (7) has a shape of a dish for depositing the collected layers (8) of the fibres (5), the apparatus being further provided with a piston for pressing the fibres (5) into the accumulator (7) and for compressing the individual layers (8) of the collected layers (8) of the fibres (5) for the purpose of mechanical strengthening of the ordered 3D structure.

11. The apparatus of claim 10 **characterised in that** the accumulator (7) is arranged rotationally around a line perpendicular to the surface of the accumulator (7) and passing through the centre of the accumulator (7) surface for turning the accumulator (7) around slightly for depositing the subsequent layer (8) of the fibres (5) settled between two adjacent electrodes (6) with the fibres (5) direction different from the direction of the fibres (5) of the preceding layer (8).

## Patentansprüche

1. Ein Verfahren zur Herstellung von zweidimensionalen oder dreidimensionalen faserigen Werkstoffen, die aus in bevorzugten Richtungen angeordneten Fasern (5) bestehen, wobei die Fasern (5) einen im Bereich von Mikrofasern bis Nanofasern liegenden Durchmesser aufweisen, wobei in dem Verfahrensschritt a)
- die Faser kontinuierlich aus einer Lösung (1) oder einer Schmelze gezogen wird und anschließend mittels eines elektrostatischen Feldes zu einem drehbaren Satz (11) von *n* leitfähigen Elektroden (6) geführt wird, wobei *n* eine natürliche Zahl ist, wobei die einzelnen Elektroden (6), aus den der Satz (11) besteht, in gleichmäßigen gegenseitigen Abständen und zugleich in demselben Abstand von der Drehungsachse des Satzes (11) von den Elektroden (6) und parallel zu dieser Achse angeordnet sind, wobei die Faser (5) auf den Satz (11) von den Elektroden (6) aufgewickelt wird, indem der Satz (11) von den Elektroden (6) in eine Drehbewegung gesetzt wird, worauf in dem Verfahrensschritt b)
- das elektrostatische Feld abgeschaltet wird und die Drehbewegung des Satzes (11) von den Elektroden (6) angehalten wird und anschließend eine aus den in dem zwischen zwei benachbarten Elektroden (6) wirkenden Feld ausgeformten Fasern (5) bestehende Schicht (8) herausgenommen wird,
**dadurch gekennzeichnet, dass** in dem nachfolgenden Verfahrensschritt c)
- der drehbare Satz (11) von den Elektroden (6) um einen Winkel von 360/n verdreht wird, dann die Schicht (8) der Fasern (5), die zwischen den zwei benachbarten, in dem sich an das das Feld, aus dem die Schicht (8) in dem vorhergehenden Verfahrensschritt b) herausgenommen worden ist, anschließenden Feld befindlichen Elektroden (6) entstanden sind, herausgenommen wird, und dieser Verfahrensschritt anschließend insgesamt n-mal wiederholt wird.

2. Verfahren nach Anspruch 1, **dadurch gekennzeichnet, dass** vor dem Verfahrensschritt c), in dessen Zuge die in dem zwischen zwei benachbarten Elektroden (6) wirkenden Feld entstehende Schicht (8) herausgenommen wird, ein Sammler (7) mäßig verdreht wird, um eine Richtung der Fasern (5) zu erreichen, die unterschiedlich von der Richtung der in der vorherhegenden Schicht (8) enthaltenen Fasern (5) ist.

3. Verfahren nach Anspruch 1, **dadurch gekennzeichnet, dass** die überlagerten Schichten (8), welche die Fasern (5) umfassen, zusammengepresst werden.

4. Verfahren nach Anspruch 3, **dadurch gekennzeichnet, dass** durch Zusammenpressen der die Fasern (5) umfassenden Schichten (8) die gewünschte räumliche Form des Endprodukts erreicht wird.

5. Verfahren nach Anspruch 4, **dadurch gekennzeichnet, dass** der aus den Fasern (5) ausgebildete Gegenstand mit einem anderen Medium eingebettet wird, wodurch ein Verbundwerkstoff entsteht, der die gewünschten Eigenschaften aufweist.

6. Eine Vorrichtung zur Herstellung von zweidimensionalen oder dreidimensionalen faserigen Werkstoffen, die aus den Fasern (5) bestehen, in dem Verfahren nach einem der Ansprüche 1 bis 5, welche Vorrichtung wenigstens eine mit einem ersten Potential verbundene Verspinnungsdüse (3), einen Satz (11) von leitfähigen Elektroden (6), die in gleichmäßigen gegenseitigen Abständen angeordnet und mit einem zweiten Potential verbunden sind, sowie einen Sammler (7) zum Sammeln der zwischen zwei benachbarten Elektroden (6) abgelagerten Fasern (5) umfasst, wobei die einzelnen Elektroden (6), die den Satz (11) bilden, in gleichmäßigen gegenseitigen Abständen und zugleich in demselben Abstand von der Drehungsachse des Satzes (11) von den Elektroden (6) und parallel zu dieser Achse angeordnet sind, **dadurch gekennzeichnet, dass**
- die Vorrichtung ausgestaltet ist, um den die Elektroden (6) umfassenden Satz (11) während des Verfahrensschritts a) in Drehbewegung zu bringen und um den Satz (11) während des Verfahrensschritts c) um einen Winkel von 360/n zu verdrehen, wobei *n* die Anzahl der Elektroden (6) in dem Satz (11) angibt,
- wobei der Sammler (7)
- gegenüber den Elektroden (6) derart angeordnet ist, dass er bewegbar in der Richtung der Längsachsen der Elektroden (6) ist, um die zwischen zwei benachbarten Elektroden (6) abgelagerten Fasern (5) sammeln zu können, und
- gegenüber den Elektroden (6) derart angeordnet ist, dass er bewegbar in der sich senkrecht zu den Längsachsen der Elektroden (6) ersteckenden Richtung ist, um vor der Einleitung des Sammelns der zwischen zwei benachbarten Elektroden (6) abgelagerten Fasern (5) in Eingriff bringbar zu sein sowie um nach der Vollendung des Sammelns der zwischen zwei benachbarten Elektroden (6) abgelagerten Fasern (5) außer Eingriff bringbar zu sein.

7. Vorrichtung nach Anspruch 6, **dadurch gekennzeichnet, dass** der Sammler (7) die Form eines Parallelogramms aufweist, dessen Breite kleiner ist als der Abstand zwischen den nächstliegenden Oberflächen eines Paares von benachbarten Elektroden (6), um zwischen die besagten benachbarten Elektroden (6) einschiebbar zu sein.

8. Vorrichtung nach Anspruch 7, **dadurch gekennzeichnet, dass** der Sammler (7) drehbar um eine sich senkrecht zu der Oberfläche des Sammlers (7) ersteckende Linie angeordnet ist und dabei durch die Mitte der Oberfläche des Sammlers (7) hindurchgeht, um zu bewerkstelligen, dass sich an der Oberfläche des Kollektors eine nachfolgende Schicht (8) der sich zwischen zwei benachbarten Elektroden (6) bildenden Fasern (5) in einer Richtung ablagert, die unterschiedlich von der Richtung der in der vorhergehenden Schicht (8) enthaltenen Fasern (5) ist.

9. Vorrichtung nach Anspruch 7, **dadurch gekennzeichnet, dass** der Sammler (7)
- eine viereckige Form aufweist, wobei die Seite des Vierecks kürzer ist als der Abstand zwischen den nächstliegenden Oberflächen eines Paares von benachbarten Elektroden (6), und
- drehbar um eine sich senkrecht zu der Oberfläche des Sammlers (7) ersteckende Linie angeordnet ist und dabei durch die Mitte der Oberfläche des Sammlers (7) hindurchgeht, um zu bewerkstelligen, dass der Sammler (7) um einen Winkel von 90° verdrehbar ist und somit die Ablagerung einer nachfolgenden Schicht (8) der sich zwischen zwei benachbarten Elektroden (6) bildenden Fasern (5) in einer Richtung ermöglicht, die sich senkrecht zu der Richtung der in der vorhergehenden Schicht (8) enthaltenen Fasern (5) erstreckt.

10. Vorrichtung nach Anspruch 6, **dadurch gekennzeichnet, dass** der Sammler (7) die Form einer Schale aufweist, die zur Ablagerung der gesammelten Schichten (8) der Fasern (5) vorgesehen ist, wobei die Vorrichtung ferner mit einem Kolben zum Hineinpressen der Fasern (5) in den Sammler (7) sowie zum Zusammenpressen der einzelnen Schichten (8), die zu den gesammelten Schichten (8) der Fasern (5) zählen, wobei der Zweck des Zusammenpressen in der Erreichung einer mechanischen Verfestigung der geordneten dreidimensionalen Struktur besteht.

11. Vorrichtung nach Anspruch 10, **dadurch gekennzeichnet, dass** der Sammler (7) drehbar um eine sich senkrecht zu der Oberfläche des Sammlers (7) ersteckende Linie angeordnet ist und dabei durch die Mitte der Oberfläche des Sammlers (7) hindurchgeht, um zu bewerkstelligen, dass der Sammler (7) verdreht wird und somit die Ablagerung einer nachfolgenden Schicht (8) der sich zwischen zwei benachbarten Elektroden (6) bildenden Fasern (5) an der Oberfläche des Sammlers in einer Richtung ermöglicht wird, die unterschiedlich von der Richtung der in der vorhergehenden Schicht (8) enthaltenen Fasern (5) ist.

## Revendications

1. Procédé de production des matériaux fibreux bidimensionnels ou tridimensionnels de fibres (5) disposées dans le sens préferé, les fibres (5) étant du diamètre s'étendant de microfibres à nanofibres, dans lequel à l'étape a)
- la fibre (5) est extraite en continu d'une solution (1) ou fondue, et tirée sur un ensemble (11) rotatif de ***n*** électrodes (6) conductrices, où ***n*** est un nombre naturel, au moyen d'un champ électrostatique, les électrodes (6) individuelles de l'ensemble (11) étant disposées à un espacement régulier l'une de l'autre et à la même distance de l'axe de rotation de l'ensemble (11) des électrodes (6) et parallèlement à celui-ci, la fibre (5) étant enroulée sur l'ensemble (11) des électrodes (6) en faisant tourner l'ensemble (11) des électrodes (6), après quoi dans l'étape b)
- le champ électrostatique est déconnecté et la rotation de l'ensemble (11) des électrodes (6) est arrêtée et une couche (8) des fibres (5) formée dans le champ entre deux électrodes (6) adjacentes est retirée,
**caractérisé en ce que** dans l'étape suivante c)
- l'ensemble (11) rotatif des électrodes (6) tourne d'un angle de 360 / ***n**,* la couche (8) des fibres (5) formée entre deux électrodes (6) adjacentes dans le champ adjacent au champ à partir duquel la couche (8) a été retirée à l'étape b) précédente, est retirée et cette étape est répétée dans le total des ***n***-fois.

2. Procédé selon la revendication 1, **caractérisé en ce qu'**avant l'étape c), où la couche (8) formée dans le champ entre deux électrodes (6) adjacentes est retirée, l'accumulateur (7) est tourné légèrement pour atteindre la direction des fibres (5) qui est différente que la direction des fibres (5) de la couche (8) précédente.

3. Procédé selon la revendication 1, **caractérisé en ce que** les couches (8) superposées des fibres (5) sont pressées ensemble.

4. Procédé selon la revendication 3, **caractérisé en ce qu'**une forme spatiale requise du produit final est formée en comprimant les couches (8) des fibres (5).

5. Procédé selon la revendication 4, **caractérisé en ce que** l'objet formé des fibres (5) est engrobé avec un autre médium, créant ainsi un matériau composite de propriétés requises.

6. Appareil pour la production de matériaux fibreux bidimensionnels ou tridimensionnels des fibres (5) pour la mise en oeuvre du procédé selon les revendications 1 à 5, comprenant au moins une buse (3) de filage reliée à un premier potentiel et l'ensemble (11) des électrodes (6) conductrices, en position frontale contre la buse, disposées à un espacement régulier l'une de l'autre et fixées à un second potentiel, et un accumulateur (7) pour collecter les fibres (5) installé entre deux électrodes (6) adjacentes, les électrodes (6) individuelles de l'ensemble (11) d'électrodes (6) étant disposées à un espacement régulier l'une de l'autre et dans la même distance de l'axe de rotation de l'ensemble (11) d'électrodes (6) et parallèles à celui-ci, **caractérisé en ce que**
- l'appareil est adapté pour faire tourner l'ensemble (11) des électrodes (6) pendant l'étape a) et pour faire tourner l'ensemble (11) de l'angle de 360/***n*** pendant l'étape c), ***n*** étant le nombre d'électrodes (6) dans l'ensemble (11) et
- où l'accumulateur (7)
- est, par rapport aux électrodes (6), disposé de façon mobile dans la direction des axes longitudinaux des électrodes (6) pour collecter les fibres (5) se trouvant entre deux électrodes (6) adjacentes et
- est, par rapport aux électrodes (6) disposées de manière mobile dans la direction perpendiculaire aux axes longitudinaux des électrodes (6) pour l'engageant pour collecter les fibres (5) se trouvant entre deux électrodes (6) adjacentes et est désengagé après avoir terminé la collecte des fibres (5) se trouvant entre deux électrodes (6) adjacentes.

7. Appareil selon la revendication 6, **caractérisé en ce que** l'accumulateur (7) a une forme de parallélogramme dont la largeur est inférieure à la distance entre les surfaces les plus proches d'un couple d'électrodes (6) adjacentes pour permettre son insertion entre lesdites électrodes (6) adjacentes.

8. Appareil selon la revendication 7, **caractérisé en ce que** l'accumulateur (7) est disposé de façon rotative autour d'une ligne perpendiculaire à la surface de l'accumulateur (7) et traversante le centre de la surface de l'accumulateur (7) pour déposer une autre couche (8) des fibres (5) se trouvant entre deux électrodes (6) adjacentes avec la direction de la fibre (5) différente de la direction des fibres (5) de la couche précédente (8).

9. Appareil selon la revendication 7, **caractérisé en ce que** l'accumulateur (7)
- a une forme carrée avec son côté plus court que la distance entre les surfaces les plus proches de deux électrodes (6) adjacentes et
- est disposé de façon rotative autour d'une ligne perpendiculaire à la surface de l'accumulateur (7) et traversante le centre de la surface de l'accumulateur (7) pour tourner l'accumulateur (7) d'un angle de 90° pour déposer la couche suivante (8) des fibres (5) placées entre deux électrodes (6) adjacentes avec la direction les fibres (5) perpendiculaire à la direction des fibres (5) de la couche précédente (8).

10. Appareil selon la revendication 6, **caractérisé en ce que** l'accumulateur (7) présente une forme d'assiette pour déposer les couches (8) collectées des fibres (5), l'appareil étant en outre muni d'un piston pour presser les fibres (5) dans l'accumulateur (7) et pour comprimer les couches (8) individuelles des couches (8) collectées des fibres (5) pour renforcer mécaniquement la structure 3D ordonnée.

11. Appareil selon la revendication 10, **caractérisé en ce que** l'accumulateur (7) est disposé de façon rotative autour d'une ligne perpendiculaire à la surface de l'accumulateur (7) et traversant le centre de la surface de l'accumulateur (7) pour faire tourner l'accumulateur (7) légèrement pour déposer la couche (8) suivante des fibres (5) se trouvant entre deux électrodes (6) adjacentes avec la direction des fibres (5) différente que la direction des fibres (5) de la couche précédente (8).
